

May 11, 1943.

J. A. LEERMAKERS ET AL

2,318,788

INCORPORATION OF COUPLERS IN NON-GELATIN EMULSIONS

Filed Oct. 26, 1940

FIG. 1



FIG. 2



JOHN A. LEERMAKERS  
SCHEURING S. FIERKE  
INVENTORS

BY *Walter M. Lewis*  
*P. Frank Smith*  
ATTORNEYS

## UNITED STATES PATENT OFFICE

2,318,788

INCORPORATION OF COUPLERS IN  
NONGELATIN EMULSIONS

John A. Leermakers and Scheuring S. Fierke,  
Rochester, N. Y., assignors to Eastman Kodak  
Company, Rochester, N. Y., a corporation of  
New Jersey

Application October 26, 1940, Serial No. 363,012  
In Great Britain December 29, 1939

7 Claims. (Cl. 95—7)

This invention relates to color couplers and to color photographic elements containing them.

In particular the invention relates to color photographic elements of the type in which a support (which may be of transparent material such as cellulose nitrate or cellulose acetate or of opaque or translucent material such as paper) carries a plurality, preferably three, of differentially color-sensitized emulsions, one or more or all of which contain color couplers, i. e., bodies which are capable of combining with the oxidation product of the developing agent used for developing the exposed silver salt to metallic silver with the production of coloring matter in the region where the silver is developed. Subsequent removal of metallic silver without removal of coloring matter leaves substantially clear transparent dye images.

It is known that in materials of this kind difficulty arises from the fact that the couplers tend to wander from the emulsions with which they are incorporated into the adjacent emulsion whereby the true color rendered is detrimentally affected. This is the case where the emulsions are cast in layers such as one upon another, or where they are dispersed in the form of differentially color-sensitized grains in a single body of a binder such as gelatin. Attempts have been made to avoid this difficulty by introducing a group into the molecules of the couplers designed to render them non-diffusing, either by increasing the molecular weight or by giving them some degree of substantivity to the gelatin.

It is therefore, an object of the present invention to provide a method for incorporating couplers in silver halide emulsions. A further object is to provide a method for incorporating couplers in non-gelatin emulsions. A still further object is to provide a method for incorporating couplers in non-gelatin emulsions so that they will not diffuse in multi-layer coatings. Other objects will appear from the following description of our invention.

These objects are accomplished by mixing with a non-gelatin emulsion such as an emulsion of silver halide in a hydrolyzed cellulose organic acid ester of approximately 19% to approximately 33% acyl content, a compound of gelatin and a coupler capable of reacting with the development product of a primary aromatic amino coupling developing agent.

In the accompanying drawing, Fig. 1 is a sectional view of a single layer photographic element made according to our invention and Fig. 2 is a

sectional view of a multi-layer photographic element made according to our invention.

In Russell and Stauffer U. S. Patent 2,282,001, granted May 5, 1942, a method for the preparation of color forming compounds non-diffusing in gelatin was described. According to the method described in that application, an acid halide of a coupler was reacted with a protein such as gelatin under conditions which produced a 10 pound of the protein and the coupler capable of jelling. This method involved the use of such reaction conditions, for example, time and temperature of reaction, that the protein was not appreciably degraded and reacted with the coupler to produce a compound of the coupler and the protein which would jell and which could be mixed with gelatin emulsions to form an emulsion capable of rendering a colored image upon suitable development.

20 It has now been found that color formers which have been combined with gelatin or other protein as described in Russell and Stauffer Patent 2,282,001, can be dispersed in emulsions of silver halide in vehicles other than gelatin and in particular in emulsions of silver halide in certain cellulose esters. The compounds, when so dispersed, have still less tendency to wander from the emulsion in which they are incorporated than in the case of gelatin emulsions. The physical dissimilarity between gelatin and cellulose esters is a distinct advantage as regards the wandering of compounds of the former from layer to layer in multi-layer coatings of the layer. The chemical 30 difficulties between the gelatin and the cellulose ester is also an improvement over dispersions of a gelatin compound in gelatin.

The dispersing medium suitable for use with our invention includes cellulose nitrate and hydrolyzed cellulose organic acid esters of approximately 19% to approximately 33% acyl content. Hydrolyzed esters having an acyl content of from 19% to 26% are particularly useful due to their high water permeability. A method for preparing dispersions of silver halide in esters of this type is described in Salo U. S. Patent 2,110,491, March 8, 1939.

The following examples, which are illustrative only, indicate methods of forming emulsions according to our invention:

*Example 1*

A coupler-gelatin compound made as described in Russell and Stauffer U. S. Patent 2,282,001, 55 comprising 10 grams of 1-acetoxy-naphthalene-

5-sulfonyl gelatin was placed in 300 cc. of cold distilled water for four hours. The water was then drained off and the gelatin coupler was melted on a steam bath to produce 160 cc. of solution. When a portion of this solution was treated with a portion of the following developer and a small amount of potassium periodate, a deep blue-green color was produced showing that the coupler was capable of forming a colored image upon treatment with the oxidation product of a coupling developer.

|                                                    |                   |        |
|----------------------------------------------------|-------------------|--------|
| 2-amino - 5 - diethylamino - toluene hydrochloride | grams             | 2.0    |
| Sodium sulfite                                     | do                | 2.0    |
| Sodium carbonate                                   | do                | 20.0   |
| Potassium bromide                                  | do                | 2.0    |
| Water                                              | cubic centimeters | 1000.0 |

80 cc. of the gelatin-coupler solution, containing 5 grams of the gelatin-coupler compound, were added to 95 cc. of a silver bromide emulsion in which cellulose acetate propionate having an acyl content of about 20% was used as the vehicle. This emulsion contained approximately 2½ grams of silver bromide. A plate was coated with the emulsion coating the dispersed gelatin coupler and, after drying and exposure, were developed in the developing solution described above. A blue-green image was produced.

*Example 2*

An emulsion made as described in Example 1 was sensitized with 5-4-(3-ethyl-2(3)-benzothiazolylidene)-2-butenylidene-3 - n - heptyl - 1 - phenyl-2-thiohydantoin to produce red sensitivity. This emulsion was coated on a plate and dried. An emulsion was then placed in a similar manner by using as the coupler 2-cyano-acetyl-naphthalene-x-sulfonyl gelatin, a magenta coupler. This emulsion was sensitized to green light with 5-[ (3-ethyl-2-(3)-benzoylidene)-ethylidene]-3-n-heptyl - 1 - phenyl-2-thiohydantoin. This emulsion was coated over the red sensitized emulsion and dried. This plate was then exposed under a step tablet to red light and to green light and to both green and red light together. The plate was then developed in the developer described in Example 1. Those areas exposed to red light produced a blue-green dye only, those areas exposed to green light yielded a magenta dye only and where mixtures of red light and green light were used for exposure, a combination of blue-green and magenta dyes was produced. Similarly a blue-sensitive emulsion, which need not be optically sensitized, and which would contain a yellow gelatin-coupler compound, could be coated over the emulsions described above to produce a complete multi-color element.

The preparation of the sensitizing dyes referred to in Example 2 is described in Brooker U. S. Patent 2,282,116, granted May 5, 1942.

Our invention will now be described by reference to the accompanying drawing. As shown in Fig. 1, 10 is a support of transparent material such as cellulose acetate or cellulose nitrate or opaque material such as paper, having thereon an emulsion layer 11 of silver halide dispersed in a water permeable cellulose ester and containing particles 12 of a gelatin coupler compound. Fig. 2 shows a multi-layer element in which the support 10 is coated with emulsion layers 13, 14 and 15 of silver halide dispersed in a water permeable cellulose ester and sensitive, respectively, to the red, green and blue re-

gions of the spectrum. The element will contain the usual yellow filter layer 16 between layers 14 and 15. Layer 13 of this element contains particles 17 of gelatin and blue-green coupler, layer 14 contains particles 18 of gelatin and magenta coupler and layer 15 contains particles 19 of gelatin and yellow coupler. This element may be developed to a colored image directly after exposure or may be developed first in a black and white developer, then developed in a color forming developer to produce colored images in the remaining silver halide of the element.

In addition to the formation of sensitive emulsions by incorporation of couplers in dispersions of silver halide in cellulose esters, filter and anti-halation layers may also be formed according to our invention by incorporating reaction products of dyes and gelatin in cellulose esters.

The examples referred to herein are understood to be for purposes of illustration only and our invention is to be taken as limited only by the scope of the appended claims.

We claim:

1. The method of preparing a color-forming photographic emulsion which comprises mixing with an emulsion of silver halide in a hydrolyzed cellulose organic acid ester of approximately 19% to approximately 33% acyl content, a compound of gelatin and a coupler capable of gelling and also capable of reacting with the development product of a primary aromatic amino coupling developing agent.

2. The method of preparing a color-forming photographic emulsion which comprises mixing with an emulsion of silver halide in a hydrolyzed cellulose acetate of approximately 19% to approximately 33% acetyl content, a compound of gelatin and a coupler capable of gelling and also capable of reacting with the development product of a primary aromatic amino coupling developing agent.

3. The method of preparing a color-forming photographic emulsion which comprises mixing with an emulsion of silver halide in a hydrolyzed cellulose acetate propionate of approximately 19% to approximately 33% acyl content, a compound of gelatin and a coupler capable of gelling and also capable of reacting with the development product of a primary aromatic amino coupling developing agent.

4. The method of preparing a color-forming photographic emulsion which comprises mixing with an emulsion of silver halide in a hydrolyzed cellulose organic acid ester of approximately 19% to approximately 33% acyl content, a naphthalene sulfonyl gelatin coupler capable of gelling and also capable of reacting with the development product of a primary aromatic amino coupling developing agent.

5. A photographic emulsion capable of producing a colored image upon development in a primary aromatic amino coupling developing agent, which comprises a hydrolyzed cellulose organic acid ester of approximately 19% to approximately 33% acyl content containing a sensitive silver halide and a compound of gelatin and a coupler capable of gelling and also capable of reacting with said developing agent.

6. A photographic emulsion capable of producing a colored image upon development in a primary aromatic amino coupling developing agent, which comprises a hydrolyzed cellulose acetate of approximately 19% to approximately 33% acetyl content containing a sensitive silver

halide and a compound of gelatin and a coupler capable of gelling and also capable of reacting with said developing agent.

7. A photographic emulsion capable of producing a colored image upon development in a primary aromatic amino coupling developing agent, which comprises a hydrolyzed cellulose acetate

propionate of approximately 19% to approximately 33% acyl content containing a sensitive silver halide and a compound of gelatin and a coupler capable of gelling and also capable of reacting with said developing agent.

JOHN A. LEERMAKERS.  
SCHEURING S. FIERKE.